

## 1

2,726,955

**SILVER HALIDE EMULSIONS CONTAINING ANTI-PLUMMING AND ANTI-BRONZING AGENTS**

Norman E. Parnell, East Brunswick Township, Middlesex County, N. J., assignor to E. I. du Pont de Nemours and Company, Wilmington, Del., a corporation of Delaware

No Drawing. Application December 19, 1952,  
Serial No. 327,049

18 Claims. (Cl. 95—7)

This invention relates to photographic silver halide emulsions and emulsion layers which have improved resistance to plumping and bronzing of developed images in photographic elements embodying such emulsions and to processes of making the same. More particularly, it relates to such emulsions and emulsion layers containing finely divided particles of an antiplumming agent suspended in wax particles.

This invention has for an objective the provision of improved photographic elements and particularly photographic papers. Another object is to improve the quality of the finished photographic image obtained when prints are dried upon hot ferrotyping equipment. A further object is to provide photographic silver halide layers which are resistant to the phenomenon known as "plumping," or "bronzing," which occurs on hot ferrotyping photographic prints and is characterized by the formation of poor image color and a decrease in image density. An additional object is to improve the effectiveness of antiplumming agents in photographic silver halide emulsion layers. Still another object is the provision of plumping-resistant photographic materials in which speed-loss and contrast-increase, encountered when employing an antiplumming agent as an emulsion adjuvant, are minimized. Other objects will be apparent from the following description of the invention.

The above objects are attained and new and useful photographic emulsions and emulsion layers are obtained by bringing into intimate mixture with the light-sensitive silver halide grains or an aqueous dispersion thereof, in a water-permeable colloid, finely divided particles of a wax containing an anti-plumming agent. The particles of the latter agent are provided with a thin skin or coating, the thickness of which varies in accordance with the proportion of wax to agent. This coating effectively prevents the anti-plumming agent from acting upon the photosensitive silver halides during storage and treatment of the exposed photographic element in aqueous processing baths, but releases the agent when the photographic element is placed in contact with the hot ferrotyping plate.

Various natural and synthetic waxes can be used for this purpose including mineral waxes, vegetable waxes, animal waxes, etc., including soft, hard and micro-crystalline paraffin waxes; ozokerite, ceresin, carnauba wax, beeswax, montan wax, synthetic waxes, e. g., seekay wax obtained by chlorinating naphthalene, chlorinated biphenyl, higher aliphatic cyanides or nitriles, higher aliphatic acid amides, methylene distearamide, ethylene distearamide and the corresponding bis amides from lauric, palmitic and oleic acid and mixtures of two or more of such amides, the synthetic wax sold under the trade name "Ceramid" by Glyco Products Co., Inc., New York, etc. The useful waxes, in general, should be solid at 25° C. and melt at the temperature used for the hot ferrotyping plate, e. g., below 100° C. The paraffin waxes are preferred.

The above waxes are water-insoluble and are not

## 2

affected by the alkaline materials or acid materials present in the usual developing, fixing and stop baths used in processing exposed photographic papers to photographic images or pictures.

- 5 In general, the procedure for inertizing an antiplumming agent consists of incorporating the anti-plumming agent in the molten wax. If the anti-plumming compound is soluble in the wax or resin, a solution may be prepared; otherwise, it is necessary to form a solution 10 using a common solvent, or a colloidal suspension with a suitable dispersing agent. In the case of 1-phenyl-5-mercaptopentetrazole and related 1-hydrocarbon-substituted 5-mercaptopentetrazoles and methylene stearamide, for example, it is possible to dissolve the anti-plumming agent directly in the liquefied wax. By melting paraffin wax and cooling carefully it is possible to disperse finely divided particles of 1-phenyl-5-mercaptopentetrazole, which is insoluble in paraffin wax, directly in the wax. However, dispersing agents, e. g., sodium p-tertiaryoctylphenoxymethoxyethyl sulfonate, aid in securing stable suspensions. The wax solution or dispersion may be dispersed in turn in water, which may contain dispersing agents, a water-permeable colloid, e. g., gelatin, forming a suspension of wax particles in which the anti-plumming agent 15 particles are coated. The water dispersion is then added to a silver halide photographic emulsion in the desired amount, coated on a suitable support, and air dried. These coatings, after receiving a standard exposure through a standard negative, are processed in the appropriate developer, acid stop and fixing solutions. The prints obtained when dried upon a hot ferrotyping plate are essentially free from plumping and exhibit no loss 20 in density, and no appreciable change in emulsion speed and contrast.
- 25 The preparation of the water dispersion of the resin solution or initial wax dispersion should be performed in a manner that will minimize leaching of the anti-plumming compound from the protective coating of wax. The use of water-insoluble solvents which have a high 30 solvent action upon the anti-plumming agent, compared to the solubility in water, is advantageous, although satisfactory coating with the anti-plumming agent or inertization is possible with certain water-soluble solvents. Coating of the agent is usually aided by concentrating the wax and anti-plumming agent in the same solvent phase. The choice of a solvent using the solute distribution laws of multiphase systems as a guiding principle aids in minimizing leaching.
- 35 The apparatus employed in preparing the water dispersions to be added to the photographic emulsion must be 40 such that the particles formed are small enough to remain dispersed for a practical period of time. Rapid mechanical stirring may be adequate in some cases. Apparatus, such as a high speed liquid blending mixer or homogenizer, may be employed. Colloid mills can be used if the 45 shearing discs are suitably spaced.
- 50 The range of particles sizes may vary over a range extending from the submicroscopic to approximately 30 microns in diameter.
- 55 In dispersing the mixture of wax and antiplumming agent directly in an aqueous colloid solution or aqueous colloid silver halide dispersion one may use small amounts of a dispersing agent. Suitable dispersing agents include sodium and potassium alkyl sulfates of 10 to 18 carbon atoms, sodium alkylsulfonates of 10 to 18 carbon atoms, 60 polyoxyethylene ethers of ring-dehydration products of a hexitol (see U. S. Patent 2,400,532), sorbitan monostearate, etc. Good dispersion can be made without agents.
- 65 While it is preferable to disperse the wax-coated particles of the anti-plumming agent in the colloid-silver halide dispersion the invention is not limited to this embodiment. Good results can be obtained by coating a 70

layer of a water-permeable colloid containing the coated anti-plumming agent directly onto a colloid silver halide emulsion layer or by bathing such an emulsion layer with a dispersion of the wax-protected anti-plumming agent.

The invention will be further illustrated but is not intended to be limited by the following examples.

#### EXAMPLE I

First, a suspension of finely-divided particles of 1-phenyl-5-mercaptoprotetrazole, having a particle size of not more than 30 microns in their largest diameter, in paraffin wax was formed by melting 200 grams of the wax, adding 2 grams of sodium p-tertiary-octylphenoxyethoxyethyl sulfonate as a dispersant and then incorporating 20 grams of the 1-phenyl-5-mercaptoprotetrazole. By cooling slowly with good agitation, a dispersion of 1-phenyl-5-mercaptoprotetrazole in the solid wax was obtained. Next, a solution consisting of 5 grams of the polyoxyethylene ether of dodecyl alcohol in 150 ml. of distilled water was prepared and added to a high-speed liquid mixer of the type described in Osiris U. S. Patent 2,109,501. A 4-gram portion of the suspension of wax-protected 1-phenyl-5-mercaptoprotetrazole particles was then added and vigorously agitated for five minutes.

A chloro-bromide emulsion (AgCl=95.2 mole per cent, and AgBr=4.8 mole per cent) was prepared by a procedure which normally yields a standard contact printing speed emulsion. Immediately before coating this emulsion upon a baryta coated paper support, 50 ml. of the wax-protected 1-phenyl-5-mercaptoprotetrazole dispersion was added to a quantity of emulsion having a silver content equivalent to that contained in 12.5 ml. of 3 N silver nitrate solution at 25° C. In all other respects the procedures for preparation and coating of contact printing paper type emulsion were followed. Control coatings were made at the same time with portions of the original emulsion, which included no 1-phenyl-5-mercaptoprotetrazole in one case, and the above wax-protected 1-phenyl-5-mercaptoprotetrazole in a second case. The coatings were dried, and samples cut and exposed to a standard negative in the standard testing set-up for contact type emulsion to obtain matched prints. All prints were developed for one minute at 20° C. in developer made by diluting 1 part of the following stock solution:

|                              |       |      |
|------------------------------|-------|------|
| Water                        | ml    | 500  |
| Metol                        | grams | 3.0  |
| Sodium sulfite (anhydrous)   | do    | 45.0 |
| Hydroquinone                 | do    | 12.0 |
| Sodium carbonate (anhydrous) | do    | 67.5 |
| Potassium bromide            | do    | 1.9  |
| Water to make 1.0 liter.     |       |      |

with 2 parts of water, rinsed in water, and fixed in the following fixer solution:

|                              |       |      |
|------------------------------|-------|------|
| Water                        | ml    | 850  |
| Sodium thiosulfate           | grams | 240  |
| Sodium sulfite (anhydrous)   | do    | 15.0 |
| Acetic acid (28%)            | ml    | 48.0 |
| Boric acid (crystals)        | grams | 7.5  |
| Potassium alum               | do    | 15.0 |
| Add water to make 1.0 liter. |       |      |

for five minutes. Processed prints from each coating were dried on a hot ferrotyp plate, a cold ferrotyp plate, and on a cheesecloth type screen to evaluate plumping. The results are tabulated as follows:

Table I

| Emulsion           | Grams 1-phenyl-5-mercaptoprotetrazole, per emulsion unit | Fog   | Relative Exposure Time (sec.) | Plummed on Hot Ferro.? | Contrast Grade |
|--------------------|----------------------------------------------------------|-------|-------------------------------|------------------------|----------------|
| Control            | none                                                     | Trace | 25                            | Yes                    | 2.0            |
| Modified with wax+ | 2.000                                                    | None  | 25                            | Slightly               | 3.0            |
| Modified with wax+ | 0.960                                                    | do    | 29                            | Very slightly          | 2.0            |
| Do                 | 0.640                                                    | do    | 21                            | No                     | 2.9            |

#### EXAMPLE II

Initially, a dispersion of finely-divided particles of 1-phenyl-5-mercaptoprotetrazole protected with paraffin wax having a melting point of 60° C. was prepared by melting 20 grams of the wax, adding 0.5 gram of an oxidized fatty acid of 12 to 20 carbon atoms as a dispersing agent, and then slowly mixing in 2 grams of the anti-plumming compound. Upon cooling slowly with good agitation, a suspension of the 1-phenyl-5-mercaptoprotetrazole in the solid wax was formed. A 3-gram portion of this mixture was then added to a solution of 6 grams of polyoxyethylene sorbitan monolaurate ("Tween 61" sold by Atlas Powder Co.) in 100 ml. of distilled water contained in a high speed mixer of the type described in U. S. Patent 2,109,501 and blended for three minutes. The dispersion thus obtained was diluted to 200 ml. and passed through a colloid mill three times, using a clearance setting of 0.002 inch and a speed of 12,000 R. P. M. The dispersion thus obtained was tested in the same manner as that described in Example I. A summary of the results is presented in Table II.

Table II

| Emulsion           | Grams 1-phenyl-5-mercaptoprotetrazole, per emulsion unit | Fog   | Relative Exposure Time (sec.) | Plummed on Hot Ferro.?        | Contrast Grade |
|--------------------|----------------------------------------------------------|-------|-------------------------------|-------------------------------|----------------|
| Control            | none                                                     | Trace | 30                            | Yes                           | 2.0            |
| Modified with      | 1.360                                                    | None  | 32                            | Moderately less than control. | 3.0            |
| Modified with wax+ | 0.680                                                    | do    | 26                            | Slightly                      | 2.0            |

#### EXAMPLE III

A solution containing 4 grams of 1-phenyl-5-mercaptoprotetrazole dissolved in 36 grams of molten, synthetic wax having a melting point of 79.5° to 80.5° C. and comprising a mixture of the amides prepared by reacting stearic acid with stearyl amines was prepared initially. Next, to 100 ml. of distilled water in a high speed mixer as described in Example II, 6 grams of sorbitan tristearate polyoxyethylene ether ("Span 65" sold by Atlas Powder Co.) were added and blended for 30 seconds. Then, 3 grams of the first molten solution were added and blended for three minutes. The resultant dispersion was diluted to 200 ml. and passed through a colloid mill three successive times, the colloid mill being set for 0.002 inch clearance and 12,000 R. P. M. The dispersion obtained was evaluated in the manner given in Example I. The pertinent results are presented in Table III.

Table III

| Emulsion           | Grams 1-phenyl-5-mercaptoprotetrazole, per emulsion unit | Fog   | Relative Exposure Time (sec.) | Plummed on Hot Ferro.?        | Contrast Grade |
|--------------------|----------------------------------------------------------|-------|-------------------------------|-------------------------------|----------------|
| Control            | none                                                     | Trace | 20                            | Yes                           | 2.0            |
| Modified with      | 1.360                                                    | None  | 33                            | Moderately less than control. | 3.0            |
| Modified with wax+ | 0.720                                                    | do    | 24                            | Slightly                      | 2.0            |

Similar results can be obtained with ether N-alkyl stearamides including those made from interaction of lauric, palmitic, oleic, and stearic acids and mixtures of two or more thereof, with the corresponding monoamines, i. e., dodecyl, etc., and mixed amines.

#### EXAMPLE IV

A solution was prepared by dissolving 2 grams of 1-phenyl-5-mercaptoprotetrazole in 20 grams of the molten

synthetic wax described in Example III. Next, a mixture of 4 grams of polyoxyethylene sorbitan monolaurate ("Tween 61" sold by Atlas Powder Co.) in 100 ml. of distilled water was prepared and blended for 30 seconds in a high-speed mixer (U. S. P. 2,101,501). A 4-gram portion of the solid wax-1-phenyl-5-mercaptopotetrazole solution was crushed and added with the mixer in motion. Blending was continued for approximately three minutes. The resultant dispersion was tested as outlined in Example I. The data obtained are given in Table IV.

Table IV

| Emulsion           | Grams 1-phenyl-5-mercaptopotetrazole, per emulsion unit | Fog   | Relative Exposure Time (sec.) | Plummed on Hot Ferro.?        | Contrast Grade |
|--------------------|---------------------------------------------------------|-------|-------------------------------|-------------------------------|----------------|
| Control            | None                                                    | Trace | 18                            | Yes                           | 2.0            |
| Modified with      | 1.360                                                   | None  | 32                            | Moderately less than control. | 3.0            |
| Modified with wax+ | 1.456                                                   | do    | 25                            | Slightly                      | 2.0            |

## EXAMPLE V

First, a solution composed of 0.75 gram of 1-phenyl-5-mercaptopotetrazole dissolved in 7.5 grams of molten stearyl stearamide was prepared and allowed to solidify. A 2-gram portion of this solid solution was then added to 100 ml. of distilled water containing 5 grams of sorbitan monolaurate and 0.5 gram of cetyl-trimethylammonium bromide as a dispersant, and blended for three minutes in a high-speed mixer (U. S. P. 2,109,501). The resultant suspension was diluted to 150 ml. and passed through a colloid mill set for 0.002 inch clearance and 12,000 R. P. M. After milling, distilled water was used to rinse the emulsifying equipment and adjust the total volume to 250 ml. Results of the emulsion evaluation of the suspensoid obtained are tabulated in the following Table V.

Table V

| Emulsion           | Grams 1-phenyl-5-mercaptopotetrazole, per emulsion unit | Fog   | Relative Exposure Time (sec.) | Plummed on Hot Ferro.? | Contrast Grade |
|--------------------|---------------------------------------------------------|-------|-------------------------------|------------------------|----------------|
| Control            | None                                                    | Trace | 23                            | Yes                    | 2.0            |
| Modified with      | 1.360                                                   | None  | 26                            | No                     | 3.0            |
| Modified with wax+ | 0.582                                                   | Trace | 25                            | No                     | 2.0            |
| Do                 | 1.456                                                   | None  | 26                            | No                     | 2.0            |
| Do                 | 0.582                                                   | Trace | 25                            | No                     | 2.0            |

## EXAMPLE VI

A second dispersion was made following the procedure given in Example I, except that ("Tween 81") was substituted for sodium p-tertiary-octylphenoxyethoxyethyl sulfonate. This dispersion was tested along with the first, so that the controls are the same. The results are also given in Table V.

In the foregoing tables an emulsion unit is defined as that quantity of emulsion having a silver content equivalent to that of 500 ml. of 3 N  $\text{AgNO}_3$  at 25° C.

The contrast grade in the foregoing tables was determined visually by comparing a print made in the standard manner with the scale of paper contrast grades used by E. I. du Pont de Nemours and Company in their control laboratory at Rochester, New York, to grade photographic paper products for trade purposes.

The above examples evidence that by coating anti-plumming agent particles with a wax one can materially reduce the degree of plumping. Moreover, the quantity of the anti-plumming agent required to give effective anti-plumming may be reduced by providing such a coating.

The invention is, of course, not limited to the use of the particular anti-plumming agent given in the foregoing examples as many other of such agents can be used with like results. Among the additional useful agents are the

- 5 1-alkyl, 1-aryl and 1-cycloalkyl-5-mercaptopotetrazoles, e. g., 1- $\alpha$ -naphthyl-5-mercaptopotetrazole, 1-cyclohexyl-5-mercaptopotetrazole, 1-methyl-5-mercaptopotetrazole, 1-ethyl-5-mercaptopotetrazole; S:S'-methylene-bis-thiuronium iodide, S:S'-ethylene-bis-thiuronium bromide, S:S'-trimethylene-bis-thiuronium bromide; 2:2'-methylenethio-bis-dihydroiminoazole dihydroiodide, 2:2'-ethylenethio-bis-dihydroiminoazole dihydrobromide, 2:2'-trimethylenethio-bis-dihydroiminoazole dihydrobromide, 2:2'-ethylenethio-bis-(4-methyldihydroiminoazole) dihydrobromide, 2:2'-trimethylene-thio-bis-(4-methyldihydroiminoazole) dihydrobromide, disodium 2:2' - ethylenethio - bis - (4-amino-6-hydroxypyrimidine), S:S'-ethylene-bis-N-ethyl-thiuronium bromide, S:S'-ethylene-bis-N:N'-diethylthiuronium bromide, S:S'-trimethylene-bis-N:N''-triethylthiuronium bromide, S:S'-ethylene-bis-N:N''-triethylthiuronium bromide, S:S'-oxylenyl-bis-thiuronium bromide, S:S'-ethylenethio-bis-(1-methyl-dihydroiminoazole) di - p - toluenesulfonate, S:S'-ethylene-bis-N-phenyl-N-methylthiuronium bromide, 4:4'-ethylene-thio-bis-(4:6-dithio-1:3:5-thio diazine, 2:2'-ethylenethio-bis-(5-thiol-1:3:4-thiodiazole), S-ethylthiuronium bromide, S-n-butylthiuronium bromide, S-cetyl thiuronium iodide, S-amidoethylthiuronium chloride, S-2-thiazylamidomethylthiuronium chloride and S-2-pyridylamidomethylthiuronium chloride, etc. Mixtures of two or more of
- 15 the anti-plumming agents can be used. They may be used with the waxes described above or mixtures of two or more of such waxes.

The proportion of anti-plumming agent to wax may vary from 1 to 25 parts by weight of the former per part 35 by weight of the latter. The optimum amounts will vary with the particular agent and wax. When the anti-plumming agent also has good anti-fogging properties it is best to keep the proportion of agent to wax in the higher portion of the above range.

40 Since waxes are insoluble in the pH ranges of the ordinary developing and fixing solutions the agents are essentially insolubilized or protected by the wax coating during aqueous processing of a photographic paper bearing an emulsion containing a wax-protected agent. The 45 amount of free or exposed anti-plumming agent can be controlled to some extent by other factors among which are proper choice of solvents, concentrations, temperature, and the severity and time of application of the shearing forces due to the dispersing equipment. It is also 50 possible to use hydrophilic colloid, e. g., gelatin solutions as the dispersion media, so that photographic emulsion wash technique may be used to remove non-protected particles, which are water-soluble. The anti-plumming agent is released by the heat of the hot ferrotype plate, which 55 melts the protective wax or resin coating.

The invention is not limited to gelatin silver halide emulsion and emulsion layers as many other water-permeable colloids can be used as the binding agent for the silver halide grains with like results. Among the additional useful materials are agar agar, alginic acid, sodium alginate, polyvinyl alcohol and its ethers and acetals including the color-former acetals of Jennings et al. U. S. P. 2,397,864, cellulose ethers, etc. partially hydrolyzed esters of cellulose, etc.

65 While the invention is particularly useful with photographic printing papers the support is not limited to paper but can be a cellulose derivative, e. g., cellulose acetate, cellulose nitrate, etc., a super polymer, e. g., nylon, polyvinyl chloride, polyethylene terephthalate, etc. These 70 supports may contain an opacifying agent or bear a coating containing such an agent so that the surface is light-reflecting and the support does not transmit light.

An advantage of this invention is that it provides a 75 simple and effective method of improving the anti-plum-

ming effect of anti-plumming agents. Another advantage is that it reduces the quantity of anti-plumming agent necessary to produce an adequate result. A further advantage is that it reduces the leaching of anti-plumming agents from water-permeable colloid silver halide emulsion layers. A still further advantage resides in the fact that the additional material involved, viz., the wax, is inexpensive. Yet another advantage is that the method of making the emulsions is simple and does not involve expensive apparatus.

As many widely different embodiments of this invention can be made without departing from the spirit and scope thereof, it is to be understood that the invention is not to be limited except as defined by the claims.

What is claimed is:

1. A colloid silver halide emulsion having dispersed therethrough particles of a wax containing an agent taken from the group consisting of anti-plumming and anti-bronzing agents, said agents being sulfur- and nitrogen-containing organic compounds having the property of preventing the formation of bronze, to plum-colored silver images upon the hot-drying of developed silver photographic images.

2. A water-permeable colloid silver halide emulsion layer having a wax in particulate form dispersed throughout such layer and having an anti-plumming agent, said agent being a sulfur- and nitrogen-containing organic compound having the property of preventing the formation of bronze- to plum-colored silver images upon the hot drying of developed silver photographic images contained in the wax particles.

3. A water-permeable colloid silver halide emulsion having dispersed therethrough particles of wax containing an anti-plumming agent, said agent being a sulfur- and nitrogen-containing organic compound having the property of preventing the formation of bronze- to plum-colored silver images upon the hot drying of developed silver photographic images, said particles having an average diameter not greater than 30 microns and said wax being solid at temperatures of 25° C. and melting at a temperature not greater than 100° C.

4. A gelatino silver halide emulsion having dispersed therethrough particles of wax containing an anti-plumming agent, said agent being a sulfur- and nitrogen-containing organic compound having the property of preventing the formation of bronze- to plum-colored silver images upon the hot drying of developed silver photographic images, said particles having an average diameter not greater than 30 microns and said wax being solid at temperatures of 25° C. and melting at a temperature not greater than 100° C.

5. A water-permeable colloid silver halide emulsion having dispersed therethrough particles of wax containing an agent taken from the group consisting of anti-plumming and anti-bronzing agents, said agents being sulfur- and nitrogen-containing organic compounds having the property of preventing the formation of bronze- to plum-colored silver images upon the hot-drying of developed silver photographic images, said particles having an average diameter not greater than 30 microns and said wax being solid at temperatures of 25° C. and melting at a temperature not greater than 100° C., the proportion of said agent to wax varying from 1 to 25 parts by weight of the former per part by weight of the latter.

6. A gelatino silver halide emulsion having dispersed therethrough particles of wax containing an anti-plumming agent, said agent being a sulfur- and nitrogen-containing organic compound having the property of preventing the formation of bronze- to plum-colored silver images upon the hot drying of developed silver photographic images, said particles having an average diameter not greater than 30 microns and said wax being solid at temperatures of 25° C. and melting at a temperature not greater than 100° C., the proportion of anti-plumming

agent to wax varying from 1 to 25 parts by weight of the former per part by weight of the latter.

7. A water-permeable colloid silver halide emulsion having dispersed therethrough particles of a water-insoluble wax containing a 1-hydrocarbon-5-mercaptopentetrazole.

8. A water-permeable colloid silver halide emulsion having dispersed therethrough particles of a paraffin wax containing a 1-hydrocarbon-5-mercaptopentetrazole.

9. A gelatino silver halide emulsion having therethrough particles of paraffin wax containing 1-phenyl-5-mercaptopentetrazole.

10. A photographic element comprising a support bearing a colloid silver halide emulsion layer wherein silver halide grains have in proximity therewith particles of a wax containing an anti-plumming agent, said agent being a sulfur- and nitrogen-containing organic compound having the property of preventing the formation of bronze- to plum-colored silver images upon the hot drying of developed silver photographic images.

20. 11. An element as set forth in claim 10 wherein the wax particles are distributed throughout the emulsion.

12. An element as set forth in claim 10 wherein the wax particles are in a separate water-permeable colloid layer disposed on the outer surface of the emulsion layer.

25. 13. A photographic element comprising a paper support bearing a water-permeable colloid silver halide emulsion layer and having dispersed therethrough particles of a wax containing an anti-plumming agent, said agent being a sulfur- and nitrogen-containing organic compound having the property of preventing the formation of bronze- to plum-colored silver images upon the hot drying of developed silver photographic images.

30. 14. A photographic element comprising a paper support bearing a water-permeable silver halide emulsion layer having dispersed therethrough particles of wax containing an anti-plumming agent, said agent being a sulfur- and nitrogen-containing organic compound having the property of preventing the formation of bronze- to plum-colored silver images upon the hot drying of developed silver photographic images, said particles having an average diameter not greater than 30 microns and said wax being solid at temperatures of 25° C. and melting at a temperature not greater than 100° C.

35. 15. A photographic printing paper comprising a baryta coated paper sheet bearing a gelatino silver halide emulsion having dispersed therethrough particles of wax containing an anti-plumming agent, said agent being a sulfur- and nitrogen-containing organic compound having the property of preventing the formation of bronze- to plum-colored silver images upon the hot drying of developed silver photographic images, said particles having an average diameter not greater than 30 microns and said wax being solid at temperatures of 25° C. and melting at a temperature not greater than 100° C.

40. 16. A photographic printing paper comprising a baryta coated paper sheet bearing a gelatino silver halide emulsion having dispersed therethrough particles of wax containing a 1-hydrocarbon-5-mercaptopentetrazole, said particles having an average diameter not greater than 30 microns and said wax being solid at temperatures of 25° C. and melting at a temperature not greater than 100° C.

45. 17. A photographic printing paper comprising a baryta coated paper sheet bearing a gelatino silver halide emulsion having dispersed therethrough particles of wax containing a 1-phenyl-5-mercaptopentetrazole, said particles having an average diameter not greater than 30 microns and said wax being solid at temperatures of 25° C. and melting at a temperature not greater than 100° C.

50. 18. The process which comprises dispersing an anti-plumming agent, said agent being a sulfur- and nitrogen-containing organic compound having the property of preventing the formation of bronze- to plum-colored silver images upon the hot drying of developed silver photographic images.

2,726,958

9

graphic images in a wax and incorporating the wax-protected particles of such agent in a light-sensitive colloid silver halide emulsion.

References Cited in the file of this patent

UNITED STATES PATENTS

2,059,829 Ward ----- Nov. 3, 1936

5 2,221,873

2,256,390

5 561,875

10

Knoefel ----- Nov. 19, 1940

Hewitson ----- Sept. 16, 1941

FOREIGN PATENTS

Great Britain ----- June 8, 1944